

# UNITED STATES PATENT OFFICE.

FEDERICO GIOLITTI, OF TURIN, ITALY, ASSIGNOR TO SOCIETA ANONIMA ITALIANA  
GIO. ANSALDO ARMSTRONG & CO., OF GENOA, ITALY.

## CASE-HARDENING PROCESS FOR ARTICLES OF IRON, STEEL, AND STEEL ALLOYS.

1,074,114.

Specification of Letters Patent. Patented Sept. 30, 1913.

No Drawing.

Application filed October 13, 1911. Serial No. 654,518.

To all whom it may concern:

Be it known that I, FEDERICO GIOLITTI, a subject of the King of Italy, and residing at 105 Corso Vittorio Emanuele, Turin, 5 Italy, have invented certain new and useful Improvements in Case-Hardening Processes for Articles of Iron, Steel, and Steel Alloys, of which the following is a specification.

This invention relates to the case hardening of objects of iron, steel or steel alloys.

In former case hardening processes the objects to be treated were heated in contact with suitable solid or gaseous carbonizing substances and maintained for a part at 15 least of the duration of the operation, out of contact with air.

The improved case hardening process according to the present invention differs from all former processes in that it consists in 20 circulating a weak air current (under determined conditions of temperature, speed of flow, and the like) through the mass of granular carbon in which the objects to be case hardened are buried, the degree of concentration of carbon in the case hardened zones being regulated by adjusting the speed of the air current.

It is impossible to state *a priori* a general rule for the determination once for all 30 of the speed of the air current necessary to obtain a determined concentration of carbon in the case hardened zone, because it is well known that the concentration besides depending on this speed, is also a function of the temperature, of the pressure and of the composition of the iron or steel under treatment, etc., so that it is impossible to give a rule covering an indefinite number of cases. It may however be affirmed that 40 in general the concentration of carbon in the case hardened zones is less when the speed of the air current which is caused to circulate through the mass of granular carbon enveloping the objects to be treated, is greater, but in every case it is necessary to 45 make trial experiments in case hardening with currents of air of different speeds in order to determine the speed of current to be adopted in order to obtain a determined concentration of carbon in the case hardened 50 zones with the iron or steel of the given composition, operating at a given temperature for a determined period of time. These trials are easy to carry out and give results 55 which it is not difficult to interpret, so that

the desired results can be easily obtained with the data thus acquired.

Two examples of the practical application of the improved process will now be given.

1. By subjecting to the case hardening 60 process according to the above described procedure, objects of mild steel containing 0.07% of carbon, for a period of two hours at 1100° C. air being circulated through the mass of granular carbon at the rate of two 65 liters per hour per square decimeter of external surface of the objects being treated, there is obtained a case hardened zone in which concentration of carbon at the outer surface is about 0.82%. 70

2. Adopting the same conditions of temperature, period, etc., but increasing the speed of the air current to the rate of twelve liters per hour per square decimeter of external surface of the steel objects being treated a concentration of carbon at the external surface of the hardened zone is 75 obtained not exceeding 0.55%.

Having thus pointed out the principle upon which is based my improved case 80 hardening process, which principle as it is easy to see is totally different from the one upon which all hitherto known case hardening processes are based, there will now be described one of the numerous methods of 85 carrying out the process. In this connection it may be stated that the improved process may be applied in different manners and with appliances which may vary according to the nature of the articles to be 90 case hardened.

The objects to be case hardened are placed in a fixed or transportable container of sheet steel or refractory material, the form and dimensions of such container depending on 95 those of the objects. Thus in many cases, as when case hardening small objects the ordinary retorts used in the preparation of illuminating gas, are quite suitable.

The container, which I shall hereinafter 100 refer to as a case hardening container, is placed in a furnace by means of which it can be heated to a constant and uniform temperature between 900° and 1150° C. The container is provided with a tightly closing 105 door for the introduction of the objects to be case hardened, and with tubes arranged in such manner as to enable a weak air current to be circulated through the container. A layer of carbon is first introduced into 110

the case hardening containers, preferably wood charcoal heated to an elevated temperature and reduced to grains or small pieces, which carbon will be herein referred to as 5 granular carbon. It is evident that the dimensions of the granular carbon and the thickness of the said layer thereof will vary with the dimensions, number and form of the objects to be case hardened. Assuming 10 that there is to be case hardened at a single operation 100 kilograms of steel articles of not too complicated form (for example cones for ball bearings, springs for bicycle wheels or the like) each weighing not more than 15 400-500 grams, it will be suitable to pound the charcoal and utilize that portion which can pass through a sieve containing 25 meshes per square centimeter but which is retained by a sieve containing 81 meshes per 20 square centimeter, the thickness of the layer of this granular carbon being about 10-15 centimeters. On the other hand if the objects to be case hardened are very much larger, say armor plates for war vessels, the 25 carbon should be used in much larger pieces and the thickness of the first layer increased to about 40-50 centimeters. The objects to be case hardened are laid on this layer of cement, spaces of about one or two centimeters being left between each object.

When the objects owing to their form or weight tend to become embedded in the carbon it will be easy to keep them in place by resting them on a piece of wire gauze. If 35 the objects are flat or elongated they can be arranged vertically. On the objects thus disposed there is scattered a quantity of granular carbon prepared as above described, sufficient to completely cover them. 40 On this second layer of carbon the other objects to be case hardened are arranged and covered with a further layer, this arrangement being repeated until the case hardening container is full.

45 The pure granular charcoal prepared in the above described manner and heated to an elevated temperature constitutes (especially when it has been used several times for case hardening after the new process) a 50 very mobile mass which packs with great facility into all the cavities of the objects, which end is assisted by gently shaking the case hardening container.

It is obvious that it will be of great advantage to use charcoal in very small granules for case hardening objects of complicated form and having small cavities, although experiment has shown that with the present process the essential carbonizing 60 agent is the gaseous mixture produced by the action of the air on the first layer of carbon, and the case hardening is effected also at these parts of the objects not in contact with the charcoal but even several centimeters away therefrom.

As soon as the case hardening container has been filled the door is closed and a weak air current is caused to flow by means of the tubes before described. As already stated the speed of the air current depends 70 upon the depth and nature of the case hardened zone which it is desired to obtain.

When the case hardening is finished the gaseous current is stopped and a door provided in the bottom of the container is 75 opened. The granular carbon then flows out owing to its own weight and is collected in order to be afterward introduced into another case hardening container. The same charcoal may thus be used many times over, 80 since only a very small quantity is consumed at the places where the air current enters the container. When the granular charcoal has been thus removed there remain in the container only the case hardened articles, which 85 can be easily taken out and tempered or subjected to other treatment. When the container has been emptied it is at once ready for a repetition of the process. In many cases, particularly when very deep zones of 90 case hardening without high concentration of carbon are desired, it is preferable not to remove all the granular carbon from the container but only a sufficient amount to leave the surface of the articles uncovered, 95 after which the heating and the circulation of air through the remaining carbon may be continued. With this procedure there is obtained in the hardened zone an exceptionally 100 uniform distribution of carbon, and the carbonizing may penetrate to great depth, for example six or seven centimeters, without the concentration of carbon ever exceeding the value attained in the first part of the 105 operation.

The gases issuing from the case hardening container may be collected in a suitable gas vessel and utilized for subsequent circulation in the case hardening container. It is unnecessary therefore to burn a small 110 quantity of granular carbon, which evidently occurs when air is directly utilized. The same result may be obtained from the beginning by passing the air through wood charcoal heated to 1000-1100° C. in a separate 115 furnace before allowing it to pass into the case hardening container.

If it is desired to have a higher degree of concentration of carbon in the case hardened zone, this may be effected by introducing 120 through suitably located tubes, larger or smaller quantities of gaseous or volatile hydro-carbons, these latter being introduced in the region of the container in which the air arrives after having passed through a 125 zone of granular carbon at least ten centimeters in thickness.

When it is desired to obtain very great uniformity of the case hardened zone over the whole surface of the articles, it is pref- 130

erable to slowly rotate the case hardening container during the operation. For the same purpose the articles while still surrounded by the granular carbon, may be 5 fixed to a revolving metal shaft passing gas tight through the wall of the case hardening container.

Having now described my invention what I claim as new and desire to secure by Letters Patent is:—

1. A process for case-hardening objects of iron, steel and steel alloys comprising the following steps; packing the objects to be treated in granular carbon in a container, 15 heating the container from an external source, passing a current of air through the carbon, and adjusting the rate of flow to obtain the desired concentration of carbon in the treated article; the temperature and 20 duration of the treatment being kept constant.

2. A process for case-hardening objects of iron, steel and steel alloys comprising the following steps; packing the objects to be 25 treated in granular carbon in a container,

heating the container to 1000° C. from an external source, passing a current of air at about atmospheric pressure through the carbon and adjusting the rate of flow of the air to obtain the desired concentration of 30 carbon in the treated article; the temperature and duration of the treatment being kept constant.

3. A process for case-hardening objects of iron, steel and steel alloys comprising the following steps; packing the objects to be treated in granular carbon, in a container, heating the container from an external source, passing a current of air and of a fluid hydrocarbon through the carbon, adjusting 40 the rate of flow of the air and of the fluid hydrocarbon; to obtain the desired concentration of carbon in the treated article.

In testimony whereof I have signed my name to this specification in the presence of 45 two subscribing witnesses.

FEDERICO GIOLITTI.

Witnesses:

GHERAN,  
C. A. FERRARI.